

## UNITED STATES PATENT OFFICE

2,211,188

MANUFACTURE OF ALTERNATING CURRENT  
RECTIFIERS OF THE DRY SURFACE CON-  
TACT TYPE

Albert Leslie Williams and Leslie Ernest Thompson, London, England, assignors, by mesne assignments, to The Union Switch & Signal Company, Swissvale, Pa., a corporation of Pennsylvania

No Drawing. Application April 26, 1939, Serial No. 270,200. In Great Britain May 14, 1938

11 Claims. (Cl. 175—366)

This invention relates to the manufacture of alternating current rectifiers of the dry surface contact type, comprising a body of metal having an oxide of the metal formed directly thereon by subjecting the body to the action of an oxidising atmosphere, and has for its object to improve the process of oxidisation whereby certain important advantages are obtained.

An important desirable quality in an oxide rectifier is that its electrical resistance in the reverse direction of current flow should be stable and not liable to appreciable creep or continuous change when voltage is applied, and experience indicates that this creep is dependent amongst other conditions, upon the amount of free oxygen occluded in the oxide film or layer after its formation.

According to the present invention a substance capable of reducing the amount of free oxygen occluded in the oxide layer during its formation is arranged to be introduced into the oxidising atmosphere employed. In particular, in the case of copper oxide rectifiers comprising a copper body or blank provided with a coating or layer of cuprous oxide formed directly thereon by heating the blank to a suitable temperature in an oxidising atmosphere, advantageous results are obtained by introduction of a small quantity of the element boron either in the combined or uncombined state into the oxidising furnace during the heat treatment of the copper blanks.

In carrying the invention into practice, the boron either uncombined or combined in the form of boric acid or borax for example, may be introduced into the oxidising atmosphere in various ways. The boron or boron compound may for instance be injected into the oxidising furnace chamber in the form of vapour or a cloud of finely divided particles. Alternatively, a suitable receptacle or reservoir containing the boron or boron compound may be located within the furnace chamber, or the copper blanks, or their supports or carriers may be immersed in a suitable solution of a boron compound prior to the oxidising process.

In order to ensure the uniform distribution of the added substance the furnace chamber employed is preferably provided with a non-porous lining and with arrangements for effecting a circulation or agitation of the oxidising atmosphere within the chamber, for example, by means of an injected stream of air or oxygen.

The addition of boron to the oxidising atmosphere in the case of copper oxide rectifiers, is found to effect a considerable reduction in the

initial reverse current and the reverse creep at all impressed voltage while the uniformity and crystalline structure of the cuprous oxide formed is much improved.

Furthermore, the undesired formation of cupric oxide is reduced, only an extremely thin superficial layer of this compound being formed.

Although the initial forward resistance of the rectifier element is increased by the use of boron to an extent dependent upon the amount of this substance employed, this disadvantage can be offset by reducing the thickness of the cuprous oxide film which is permissible owing to its superior quality and to the small amount of cupric oxide formed as above explained.

The amount of boron utilised will evidently depend upon particular conditions, but is in any case extremely small relative to the amount of oxygen in the oxidising atmosphere.

It will be understood that similar advantageous results may probably be obtained by the addition of substances other than boron which has however been definitely determined to be particularly suitable in the case of copper oxide rectifiers. The invention is however not limited in this and other respects to the particular processes and arrangements above described by way of example.

Having now particularly described and ascertained the nature of our said invention and in what manner the same is to be performed, we declare that what we claim is:

1. The process for manufacturing a copper oxide rectifier which comprises subjecting a copper body to the action of an oxidizing atmosphere into which the element boron in a combined or an uncombined state has been introduced to reduce the amount of free oxygen occluded in the oxide layer during its formation.

2. The process for manufacturing a copper oxide rectifier which comprises subjecting a copper body to the action of an oxidizing atmosphere into which boron or a boron compound has been introduced in the form of a vapor or cloud to reduce the amount of free oxygen occluded in the oxide layer during its formation.

3. The process for manufacturing a copper oxide rectifier which comprises heating a copper body in an oxidizing atmosphere in a furnace having located in the oxidizing chamber a receptacle containing boron or a boron compound.

4. The process for manufacturing a copper oxide rectifier which consists in subjecting a copper body to the action of an oxidizing atmosphere while mounted on a support or car-

rier which has previously been immersed in a solution of a boron compound.

5. The process for manufacturing a copper oxide rectifier which consists in subjecting a copper body to the action of an oxidizing atmosphere into which borax or boric acid has been introduced.

6. The process for manufacturing a copper oxide rectifier which consists in heating a copper body in a furnace in an oxidizing atmosphere into which boron or a boron compound has been introduced, the oxidizing atmosphere being circulated or agitated by means of an injected stream of air or oxygen.

10 7. The process for manufacturing a copper oxide rectifier which consists in subjecting a copper body to the action of an oxidizing atmosphere into which boron or a boron compound has been introduced to effect a reduction in the initial reverse current at all impressed voltages.

15 8. The process for manufacturing a copper oxide rectifier which consists in subjecting a copper body to the action of an oxidizing atmosphere into which boron or a boron compound

has been introduced to effect a reduction in the reverse creep at all impressed voltages.

9. The process for manufacturing a copper oxide rectifier which consists in subjecting a copper body to the action of an oxidizing atmosphere into which boron or a boron compound has been introduced to improve the uniformity and crystalline structure of the cuprous oxide which is formed.

10 10. The process for manufacturing a copper oxide rectifier which consists in subjecting a copper body to the action of an oxidizing atmosphere into which boron or a boron compound has been introduced to reduce the formation of cupric oxide.

15 11. The process for manufacturing a copper oxide rectifier which consists in subjecting a copper blank to the action of an oxidizing atmosphere into which has been introduced boron in an amount which is extremely small relative to the amount of oxygen in the oxidizing atmosphere.

ALBERT LESLIE WILLIAMS.

LESLIE ERNEST THOMPSON. 25